

## UNITED STATES PATENT OFFICE.

NEWTON H. SCHNEIDER, OF SALINAS, CALIFORNIA.

## ACID-RESISTING COMPOUND.

No Drawing.

Application filed April 20, 1925. Serial No. 24,677.

My invention is a composition of matter forming a hand protection from acids. An object of my invention is to provide a mixture of ingredients which will form a good covering body for the hands, will remain thereon without becoming rubbed off, except when it is desired to remove the composition, and further to form a composition which will have a neutralizing action on acids. My composition is of particular use in storage battery stations.

My composition is an improvement over my application for an acid resisting compound, Serial No. 8,293, filed Feb. 10, 1925. In this composition I use a large proportion of a covering agent such as used in paints and preferably use white lead. This is diluted with an evaporating oil such as gasoline and baking soda, and after this mixing resin is added. To maintain the composition in the desired consistency I mix a small amount of castor-oil, eucalyptus-oil and alcohol.

My preferred composition is made substantially as follows:—and in substantially the following proportions:—for instance, one-third pound of white lead which is thinned by mixing it in the proportion of ninety-two per cent of the white lead to eight per cent of linseed oil. When the white lead has been thoroughly ground in the oil, it is mixed with a light solvent such as a very quick evaporating gasoline, about ten ounces being used. The whole mixture so far produced has added thereto, while being mixed and stirred, baking soda of the quantity of one pound. This is kept well mixed.

Commercial resin such as a turpentine resin to the quantity of one-half pound is heated until it will flow readily when one-quarter of an ounce of castor oil is added. This resin and castor-oil mixture is removed from the fire and the white lead, as thinned with the gasoline, is mixed therewith. This combined mixture is stirred for about half a minute and then at intervals of about half a minute until it stops "working" which for the quantity usually takes about ten minutes. In this operation it will become stiff and grainy to prevent which alcohol to the quantity of about ten ounces and one quarter of an ounce of eucalyptus-oil is added before it becomes too stiff to stir.

Most of the gasoline evaporates in the

heating and mixing operation, but the oils and the alcohol maintain the composition as a thin paste. It is preferable to use grain alcohol. When this is applied to the hands it will dry quickly, leaving a thin film which will wear for a long time in ordinary use of the hands in handling storage batteries, etc. The paste thoroughly protects the hands, particularly from sulphuric and hydrochloric acid. My composition may be restated to comprise the following ingredients in the proportions named, approximately:—

White lead one-third of a pound, baking soda (bicarbonate of soda)  $\text{NaHCO}_3$ , 1 70 pound, commercial resin one-half pound, one-quarter ounce castor-oil, one quarter-ounce eucalyptus-oil, and ten ounces of grain alcohol, (ethyl alcohol). The resins used may be of the colophony or copal type 75 or other suitable light resins.

The above mentioned composition may be considerably changed in proportions and other ingredients may be added. Also for convenience the hands may be covered with 80 vaseline before the mixture is applied.

Having described my invention, what I claim is:—

1. The method of forming an adherescent acid proof composition comprising mixing 85 white lead with linseed oil and thinning with gasoline, adding baking soda thereto and mixing, and as a separate step heating resin and adding thereto castor oil, combining the white lead and baking soda mixture 90 with the heated resin and mixing, and finally thinning with alcohol and eucalyptus oil.

2. The method of claim 1, in which white lead is used in the proportion of one-third 95 of a pound, the baking soda one pound, and the resin one-half pound.

3. An acid proof composition comprising white lead, baking soda, commercial resin and alcohol to thin the mixture, and in addition, a small amount of castor oil and a small amount of eucalyptus oil.

4. An acid proof composition comprising white lead one-third of a pound, baking soda one pound, commercial resin one-half 105 pound, castor oil one-fourth ounce, eucalyptus oil one-fourth ounce and alcohol sufficient to form a paste.

In testimony whereof I affix my signature.

NEWTON H. SCHNEIDER.